

## UNITED STATES PATENT OFFICE

2,262,822

SAFETY PAPER AND THE MANUFACTURE  
THEREOF

Francis L. Simons, Montclair, N. J., assignor to  
George La Monte & Son, Nutley, N. J., a corpora-  
tion of New Jersey

No Drawing. Application September 28, 1938,  
Serial No. 232,082

21 Claims. (Cl. 91—67.95)

This invention relates to safety paper including fraud-preventing writing material made of paper or other substance or composition adapted for printing or lithographing or for the inscription of writing thereon and for use, for example, in the manufacture of checks, drafts, bonds, stock certificates or other instruments which it is desired to have protected against fraudulent alteration. This invention also relates to methods of making such paper.

There are many chemical substances which are known and which have the property, when incorporated with paper during the manufacture thereof or by impregnation therein or superficial application thereto, of developing a disfiguring stain upon the application of a chemical ink eradicator thereto by changing from a colorless to a colored substance, by becoming more intensely colored or by change in color or the like when the chemical ink eradicator is applied to the paper. The developed stain that results upon application of a chemical ink eradicator to the paper makes obvious any attempt by means of a chemical ink eradicator to alter or tamper with the paper. Some chemicals such as manganese sulphate, iodides, etc., change color when a bleaching agent is applied thereto but can readily be converted back to their original condition by application of a reducing agent. Other chemicals, however, such as the chemicals specifically mentioned hereinbelow after having their color changed by the application of a chemical ink eradicator thereto cannot be readily reduced to their original color and afford a record of attempted alteration of the paper that is substantially permanent. It is substances of the latter type which are called in the safety paper art and which are referred to herein as "stain-producing" substances.

A considerable number of organic amines are known for their property of being stain-producing substances. The use of anilin or a salt of anilin such as anilin chloride is described in Patent No. 1,172,414. In Patents Nos. 1,536,861 and 1,535,863 the use of primary amines such as benzidine, toluidin, dianisidine, and diphenylamine and their derivatives is described. In Patent No. 1,839,995 aryl substances referred to therein as "guanidine substances," e. g., diphenyl-guanidine, are described as stain-producing substances for use in safety paper. In Patent No. 2,061,632, there is disclosed a large number of amino-aryl-thiazoles, reference being made particularly to 1-amino-aryl-thiazoles in which the amino-nitrogen is directly bonded to the carbon

of the thiazole ring and has at least one free amino-hydrogen and in which the aryl group contains at most two benzene rings.

It is a purpose of this invention to incorporate stain-producing substances such as the stain-producing amines in safety paper in such a way that thorough impregnation is facilitated while at the same time effecting a very permanent incorporation of the substance in the paper. It is a further purpose of this invention to incorporate in safety paper acidic derivatives of stain-producing amine substances without adversely affecting the quality and ageing characteristics of the paper. It is a further purpose of this invention to incorporate stain-producing amine substances in safety paper in conjunction with ferrocyanide as an ink-fixing substance in such a way that the ferrocyanide does not decompose prematurely and discolor the paper.

20 Ferrocyanides, when incorporated in safety paper have the property of forming with iron compounds in ink certain deeply-colored compounds known as Prussian blue, the exact chemical nature of which is not certain and may vary 25 to some extent, depending upon the proportions and character of the reacting substances. Prussian blue is highly resistant to ink eradicators in general use at the present time. The most commonly used ink eradicators have a chlorine 30 bleach as a basis. Another type of eradicator has potassium permanganate as a basis. The latter eradicator is normally followed in actual use by the application of some reducing agent such as sodium bisulphite to clean up the manganese 35 dioxide deposited during the application of the permanganate. The Prussian blue formed by writing with ordinary iron-containing ink on safety paper prepared with a ferrocyanide is resistant to the action of either of the eradicators 40 referred to. The Prussian blue is especially resistant to the potassium permanganate type of eradicator. While the Prussian blue is also resistant to a chlorine bleach type of eradicator when the color has been developed to a relatively 45 pronounced degree, faint coloration such as that produced when a very small amount of ferrocyanide is incorporated with safety paper can be affected to some extent by the chlorine bleach type of ink eradicator.

50 The stain-producing amine substances mentioned above react merely with the chlorine bleach type of eradicator to produce disfiguring stains. They do not react with the potassium permanganate type of eradicator to produce discoloration.

The stain-producing amine substances which have been mentioned above are commonly used in a water-insoluble condition. The stain-producing amine substances when so used are generally incorporated with the pulp in the beater during the manufacture of the safety paper. This method of incorporating the chemical in the safety paper is not altogether satisfactory inasmuch as there is considerable loss of the safety chemical during the formation of the paper from the pulp. Moreover, it is frequently desirable to treat paper that has already been manufactured so as to make it sensitive to chemical ink eradicator and this is difficult when a water-insoluble chemical is to be used.

There are water-soluble forms of stain-producing amine substances, the water-soluble acid salts of such substances being the most common, e. g., the hydrochloride. Other acid salts such as the other halide salts and salts of organic acids such as the acetates and formates are water-soluble. Benzidine hydrochloride, 1-amino-5-chlorobenzol-thiazole-hydrochloride and diphenyl guanidine acetate are examples of water-soluble stain-producing substances. However, the majority of the stain-producing amine substances, when in the form of a water-soluble acid salt, for example, are not stable in the presence of light and tend to decompose so as to prematurely discolor the safety paper. Moreover, the water-solubility of such substances makes it possible to wash such substances out of the safety paper, thus destroying the effectiveness of the safety paper. The fact that stain-producing amine substances can be successfully washed out of safety paper is a serious drawback to the effectiveness of the protection afforded by these materials.

According to one of the features of this invention a stain-producing substance such as a stain-producing amine is incorporated in safety paper while in a water-soluble acidic form and is converted into a water-insoluble form while incorporated in the safety paper by neutralizing the acidity of the substance. For example, a stain-producing amine substance is incorporated in the safety paper in the form of a water-soluble acid salt and, while it is incorporated in the safety paper, is treated to transform it into a water-insoluble stain-producing amine substance by neutralizing the acidity of the acid salt added to the safety paper. Other stain-producing substances such as stain-producing thioureas and their amino-derivatives may be incorporated in a similar way.

It is another feature of this invention that the neutralization of a water-soluble acid salt of a stain-producing amine substance is accomplished while it is incorporated in the safety paper by means of a buffer mixture. The buffer is effective to overcome the acidity of the stain-producing substance and has the great advantage of not being injurious in any way to the paper.

This invention may be illustrated, for example, in connection with the substance 1-amino-5-chloro-benzo-thiazole. This substance while insoluble in water, is water-soluble when in the form of the hydrochloride. According to this invention 1-amino-5-chloro-benzo-thiazole hydrochloride in aqueous solution is added to safety paper and then is transformed to insoluble form. For example, the hydrochloride is added to safety paper which contains a buffer such as a mixture

of mono-sodium phosphate and di-sodium phosphate or a mixture of borax or boric acid, or is added to the paper first, the paper thereafter being treated with the buffer. In either event the 1-amino-5-chloro-benzo-thiazole-hydrochloride while incorporated in the safety paper is transformed by the buffer from the water-soluble acid salt to a water-insoluble form. This is of advantage for the reason mentioned above, namely, that while the water-soluble hydrochloride is readily incorporated in the safety paper, it is rendered insoluble so that it is very difficult to remove the stain-producing substance from the paper by washing the paper with water. It is of even greater practical importance that the aging quality of the paper is improved. When the 1-amino-5-chloro-benzo-thiazole-hydrochloride is applied to the paper, it includes the hydrochloric acid forming part of the molecule and in addition some free hydrochloric acid which is necessary for the purpose of keeping this substance in solution. The solution as applied to the paper usually has a pH value below 4 and usually has a pH value of about 3. This causes the paper which is normally somewhat acid anyway to be removed from the bath in a distinctly acid condition. This additional acidity of the paper has a tendering effect upon the paper. The age resistance of the paper can be improved by increasing the pH value to about 5.5 and even a lesser degree of acidity than this is to be preferred for papers designed for long life.

The neutralization by means of a buffer of the acidity imparted to safety paper as a result of the addition to the paper of an acid salt of a stain-producing amine substance is distinctly preferable according to this invention. By causing the acid salt to react with the buffer, it is not necessary to make the paper distinctly alkaline at any time or to treat the paper with strongly alkaline substances, nor is it necessary to run the danger of under- or over-neutralizing the paper. While it is within the scope of this invention to neutralize the acidity of an acid salt of a stain-producing amine substance while the substance is incorporated in the paper by means of an alkali such as soda ash or a dilute caustic alkali, neutralization in this manner is regarded as much less desirable than neutralization accomplished by a buffer mixture. When a straight alkali is used, it is injurious to many types of paper and is essentially injurious to paper which has been sized with the usual rosin sizing. Moreover, care has to be exercised in controlling the amount of alkali that is used.

I have found that a ferrocyanide may be successfully incorporated in safety paper together with a stain-producing amine substance. Ferrocyanides tend to be unstable standing by themselves or in the presence of an acid when applied to safety paper, with the result that the ferrocyanide decomposes so as to cause premature discoloration of the paper. In my Patent No. 2,037,937, the stabilization of ferrocyanides incorporated in safety paper is described. The acidity of an acid salt of a stain-producing amine substance tends to cause premature decomposition of ferrocyanide applied to safety paper. I have found, however, that by incorporating a buffer with safety paper it is possible to make a stable safety paper which has been treated both with a water-soluble acid salt of a stain-producing amine and with a ferrocyanide.

The use of a buffer containing alkali metal

phosphate (including ammonium phosphate) is preferred inasmuch as the phosphate radical has been found to exercise a specific stabilizing effect on ferrocyanide as I have pointed out in my Patent No. 2,037,937. While I prefer to employ a mixture such as a mixture containing a major proportion of disodium phosphate and a minor proportion of monosodium phosphate, it is apparent that the disodium phosphate may be used by itself as a buffer to counteract the acidic effect of an acid salt of a stain-producing amine. Tri sodium phosphate may also be used but is normally less desirable than the disodium phosphate due to its greater degree of alkalinity.

A safety paper that contains a stain-producing amine substance and a ferrocyanide is extremely effective against all types of chemical ink eradicators that may be applied thereto. While the stain-producing amine does not react with the permanganate type of ink eradicator, the ink-fixing effect resulting from the reaction of the ferrocyanide with ink containing iron such as the ordinary blue-black iron gallotanate writing ink is extremely resistant to the permanganate type of ink eradicator and affords very effective protection, even when the ferrocyanide is present in only a relatively small amount. If the chlorine bleach type of ink eradicator is applied to the safety paper, the stain-producing amine substance immediately produces a discoloration or stain of a permanent character that shows that the paper has been tampered with and in addition the ink-fixing action of the ferrocyanide affords added protection when this type of ink eradicator is used. Therefore, a high degree of protection is afforded against both the permanganate type and against the chlorine bleach type of chemical ink eradicator. Moreover, due to the presence of the acid-alkali buffer in the paper, the stain-producing amine substance occurs in a water-insoluble condition and cannot be washed out of the paper.

It is also of great practical importance that the paper cannot be treated so as to wash out the safety chemicals. It has been mentioned above that stain-producing amine substances can be washed out of safety paper containing such substances in water-soluble form by washing the paper with water. Even when these substances are in water-insoluble form they can be washed out of safety paper by using dilute acid. For example, substances such as benzidine or 1-amino-5-chlor-benzo-thiazole are soluble in dilute hydrochloric acid and substances such as guanidine substances are soluble in dilute acetic acid. When, however, a ferrocyanide stabilized by a buffer is present in addition to the stain-producing substance, it is impossible to wash out the stain-producing substance. If the paper is washed with a dilute acid, the acid immediately causes the ferrocyanide to turn dark blue and to reveal the attempt to alter the paper. Therefore, the new paper of this invention, due to the combination of safety chemicals used, not only is effective against the different types of chemical ink eradicators which might be used, but also is effective against attempts to remove the safety chemicals from the paper and affords much more effective protection than that which has been regarded as possible heretofore.

In the practice of the invention using ferrocyanides, the soluble ferrocyanides are preferable, namely, the ferrocyanides of the alkali metals (including ammonium) and of alkaline earths. The ferrocyanides of sodium and potassium are

regarded as being particularly effective and are relatively inexpensive.

A further understanding of the preparation of safety paper according to this invention will be apparent from the following specific example which is illustrative of the practice of this invention. The paper is first treated with an aqueous solution of a water-soluble acid salt of a stain-producing amine substance, e. g., 1-amino-5-chloro-benzo-thiazole-hydrochloride. A solution of about  $\frac{1}{4}\%$  to 2% concentration of this substance is suitable for the purpose. The paper then may be dried or merely passed between squeeze rolls so as to press out its excess moisture and so as to make the surface of the paper free of the solution. If the paper is not completely dried it is preferable to not only pass the paper between the squeeze rolls but also over a drying drum so that the surface of the paper may be free of excess solution of acidic character. The paper is then passed through a bath containing about 5% of sodium ferrocyanide, about 12% of disodium phosphate, and about 1% of monosodium phosphate. After treating the paper with this second bath, the paper is passed between squeeze rolls so as to remove excess solution and then is dried. The paper is then ready for use although further finishing, printing or ornamentation as desired may be applied to the paper. The finished paper preferably has a pH of about 6.0 to about 7.0 although satisfactory results are also obtained when the pH value is about 6.2 to about 7.3; but these limits are not to be regarded as absolutely essential to the practice of the invention. In the foregoing example, the proportions given are based on the weight of the fully hydrated commercial salts that are added to the bath. The bath containing ferrocyanide and mono- and disodium phosphates has a pH value of about 7.0 to 7.4 when made up.

The sequence of operations mentioned above is regarded as preferable from the point of view of effectiveness and economy although the order in which the chemicals are added to the paper may vary. For example, the ferrocyanide and phosphate may be added to the paper prior to the treatment of the paper with the acid salt of the stain-producing amine substance. In such case, the acidity of the acid salt is neutralized as the salt becomes incorporated with the paper and while the salt is within the paper. Further in this connection, the treatment of the paper with a buffer may be performed as a separate step at any stage in the process. It is preferable, however, not to postpone adding the buffer until after both the acid salt of the stain-producing amine substance and the ferrocyanide are incorporated.

While it is normally preferable to apply the stain-producing amine substance or ferrocyanide or both uniformly throughout the body of the sheet in the manner above described, the solution can, of course, be applied in any other manner as by spraying the sheet with the solution, applying the solution locally by printing or otherwise, or in any other suitable manner. Whether the substances are applied through the paper or at the surface, the same are to be regarded as incorporated with the safety paper.

A stain-producing amine substance can be incorporated at the time the paper is tub sized by mixing the substance with the sizing bath. This substance can also be included in a dye bath and incorporated with the paper during the application of the dye to the paper.

When the materials are applied in the manner described in the foregoing example it will be found that the finished paper contains about  $\frac{1}{4}\%$  to about 2% of the ferrocyanide since the paper tends to take up about  $\frac{1}{5}$  of the proportion of ferrocyanide and stabilizing chemical, i. e., the phosphate that is contained in the bath. There will likewise be about 1% to about  $\frac{1}{2}\%$  of the stain-producing amine. When these two substances are used together it is desirable to have in the safety paper an amount of alkali metal phosphate or other buffer material corresponding to about 50% to about 300% of the combined ferrocyanide and amine substance in the paper. The amount of ferrocyanide that is incorporated in the paper may be increased to about 5%, the maximum amount that the paper retains when impregnated with a saturated solution of a ferrocyanide. The proportion of stain-producing amine that is used may also be increased considerably, e. g., to about 1.0% by applying a more concentrated solution thereof to the paper. In general the more ferrocyanide or stain-producing substance that is used, the more vigorous will be the ink-fixing property of the ferrocyanide and the stain-producing property of the amine substance. For purposes of economy it is preferable to use amounts such as those recommended above, however.

While it is preferable to incorporate the ferrocyanide in the paper, the ferrocyanide may be omitted. In such case the procedure mentioned in the foregoing example may be followed, using the disodium phosphate and mono-sodium phosphate mixture to convert the 1-amino-5-chloro-benzo-thiazole-hydrochloride to an insoluble form. When the ferrocyanide is omitted, however, the advantages which result from the combined presence of stain-producing substance and ferrocyanide and which have been referred to above, are also omitted. While it is preferable to introduce the stain-producing substance in water-soluble form and convert it while incorporated with the paper to a water-insoluble form and combine the stain-producing compound in insoluble form with a ferrocyanide, the stain-producing compound in insoluble form may be incorporated with the paper, as by mixing it with the pulp in the beaters, and thereafter adding the ferrocyanide to the paper to achieve the advantages that result from the combined presence of a stain-producing substance and a ferrocyanide in the finished paper.

While this invention has been described in connection with specific examples, it is to be understood that this has been done in order to illustrate the practice of this invention and the scope of this invention is to be governed by the language of the following claims.

I claim:

1. A method of making safety paper which comprises incorporating with paper a water-soluble acid salt of an organic aryl amine adapted to react with a chlorine bleach to produce a stain and converting said substance to a water-insoluble form by neutralizing the acidity of said salt.

2. A method of making safety paper which comprises treating paper with a water-soluble acid salt of an organic aryl amine adapted to react with a chlorine bleach to produce a stain, a ferrocyanide and a buffer, said acid salt being neutralized by the action of said buffer while incorporated in said paper and thereby converted into water-insoluble form and said ferrocyanide

being in the presence of said buffer when said organic amine is contacted therewith.

3. A method of making safety paper which comprises incorporating in paper a solution of a water-soluble acid salt of a stain-producing amino-aryl-thiazole substance and neutralizing the acidity of said substance to convert it into a water-insoluble form while said substance is incorporated with said paper.

4. A method of making safety paper which comprises incorporating a solution of a water-soluble acid salt of a stain-producing amino-aryl-thiazole in paper containing a buffer.

5. A method of making safety paper which comprises incorporating in paper a solution of a water-soluble acid salt of a stain-producing amino-aryl-thiazole and then treating the paper containing said incorporated acid salt with a solution containing a buffer.

6. A method of making safety paper which comprises incorporating in paper a solution of a water-soluble acid salt of a stain-producing amino-aryl-thiazole and then treating the paper containing said incorporated acid salt with a solution containing a buffer and a water-soluble ferrocyanide.

7. A method of making safety paper which comprises incorporating in paper a solution of a water-soluble acid salt derivative of benzidine and neutralizing the acidity of said salt to convert it into a water-insoluble form while the substance is incorporated in said paper.

8. A method of making safety paper which comprises incorporating in safety paper a hydrochloride of an organic aryl amine adapted to react with chlorine bleach to produce a stain, a ferrocyanide and a buffer, said hydrochloride being neutralized by action of said buffer while incorporated in said paper and said ferrocyanide being in the presence of said buffer when said hydrochloride is contacted therewith.

9. A method of making safety paper which comprises incorporating in safety paper 1-amino-5-chloro-benzo-thiazole hydrochloride, an alkali metal phosphate and a ferrocyanide.

10. A safety paper having incorporated therewith a water-insoluble organic aryl amine adapted to react with a chlorine bleach to produce a stain, a ferrocyanide, and a buffer, the pH value of the paper being between about 6.2 and about 7.3.

11. A safety paper having incorporated therewith a water-insoluble organic aryl amine adapted to react with a chlorine bleach to produce a stain, a ferrocyanide and a buffer.

12. A safety paper having incorporated therewith a water-insoluble organic aryl amine adapted to react with a chlorine bleach to produce a stain, a ferrocyanide, and an alkali metal phosphate.

13. A safety paper having incorporated therewith a water-insoluble organic aryl amine adapted to react with a chlorine bleach to produce a stain, a ferrocyanide, and an alkali metal phosphate, the phosphate being about 50% to about 300% of the combined amine and ferrocyanide.

14. A safety paper having incorporated therewith a stain-producing amino-aryl-thiazole, a ferrocyanide, and an alkali metal phosphate.

15. A safety paper having incorporated 1-amino-5-chloro-benzo-thiazole in insoluble form in the presence of a buffer and a soluble ferrocyanide.

16. A safety paper having incorporated 1-amino-5-chloro-benzo-thiazole in insoluble form

in the presence of an acid-alkali buffer and a soluble ferrocyanide, the pH value of the paper being about 6.2 and about 7.3.

17. A safety paper having incorporated therein a substance adapted to react with a chlorine bleach to produce a stain, said substance being selected from the group consisting of anilin, anilin chloride, benzidine and its derivatives that contain the benzidine nucleus, tolidin and its derivatives that contain the tolidin nucleus, dianisidine and its derivatives that contain the dianisidine nucleus, diphenylamine and its derivatives that contain the diphenylamine nucleus, aryl guanidine substances, and 1-amino-aryl-thiazoles in which the amino-nitrogen is directly bonded to the carbon of the thiazole ring and has at least one free amino-hydrogen and in which the aryl group contains at most two benzene rings; and also having incorporated therein a ferrocyanide and a buffer.

18. A safety paper having incorporated therein benzidine, a water-soluble ferrocyanide, and a buffer, the pH value of the paper being between about 6.2 and about 7.3.

19. A method of making safety paper which comprises incorporating with paper in water-soluble acidic form a substance adapted to react with a chlorine bleach to produce a stain,

said substance being selected from the group consisting of anilin, anilin chloride, benzidine and its derivatives that contain the benzidine nucleus, tolidin and its derivatives that contain the tolidin nucleus, dianisidine and its derivatives that contain the dianisidine nucleus, diphenylamine and its derivatives that contain the diphenylamine nucleus, aryl guanidine substances, and 1-amino-aryl-thiazoles in which the amino-nitrogen is directly bonded to the carbon of the thiazole ring and has at least one free amino-hydrogen and in which the aryl group contains at most two benzene rings; and converting said substance to a water-insoluble form while the substance is incorporated with the safety paper by neutralizing the acidity of the substance.

20. A safety paper having incorporated therein diphenylamine, a water-soluble ferrocyanide, and a buffer, the pH value of the paper being between about 6.2 and about 7.3.

21. A method of making safety paper which comprises incorporating in paper a solution of a water soluble acid salt derivative of diphenylamine and neutralizing the acidity of said salt to convert it into a water-insoluble form while the substance is incorporated in said paper.

FRANCIS L. SIMONS.

CERTIFICATE OF CORRECTION.

Patent No. 2,262,822.

November 18, 1941.

FRANCIS L. SIMONS.

It is hereby certified that error appears in the printed specification of the above numbered patent requiring correction as follows: Page 1, first column, line 44, for the patent number "1,536,861" read --1,535,861--; and second column, line 36, strike out "by"; page 2, second column, line 2, for "borax or" read --borax and--; page 4, second column, line 36, claim 8, insert "a" before "chlorine"; page 5, first column, line 3, claim 16, after "being" insert,--between--; and that the said Letters Patent should be read with this correction therein that the same may conform to the record of the case in the Patent Office.

Signed and sealed this 23rd day of December, A. D. 1941.

(Seal)

Henry Van Arsdale,  
Acting Commissioner of Patents.